

## UNITED STATES PATENT OFFICE.

FREDERICK M. VENZIE, OF PHILADELPHIA, PENNSYLVANIA.

## PLASTER-BLOCK COMPOSITION.

No Drawing.

Application filed May 18, 1923. Serial No. 639,973.

This invention has relation to compositions for use in building walls, partitions, ceilings and the like and is primarily designed to supplant plaster-board as now commonly used for the purpose.

The leading object of the present invention is to provide a novel form of composition from which may be readily molded plaster-blocks of light, strong, durable and comparatively cheap construction, the texture of which blocks is relatively soft, yet tough, as distinguished from hard and brittle. A further object is to provide a plaster-block composition characterized by water proofing, sound proofing and fire proofing qualities. With these and other objects in view the invention consists of the improvements hereinafter described and finally claimed.

In practice the composition may be prepared in several different ways according to results desired and uses to which the composition is to be put.

According to one mode of procedure I take from one-half to one part of finely divided saw-dust and mix therewith, in a dry state about one part of plaster-of-Paris. To these ingredients when thoroughly mixed dry I add about one part of cool water and thoroughly mix all together. From such composition blocks may be readily molded in contradistinction to compacting by hydro-press or other method. A block formed of this composition is light, strong and durable; is very cheap as compared to plaster-board; is relatively soft, yet tough and efficient for the purposes desired and may be readily cut to desired size.

In the event that the above described composition requires a binder I prefer to add to the water used about five per cent of liquid glue. In addition to forming a binder the glue acts to prevent "rapid suction" when plaster is being applied to a partition or the like formed of blocks made from the composition under discussion.

Should it be desired to harden and strengthen blocks as made from my composition I may add about five per cent of dextrine to the composition.

By adding to the composition about ten <sup>30</sup> per cent of silicate of soda the same is rendered waterproofing and fire proofing in quality and since a block made from my composition is sound proofing these additional qualities make for a very efficient and <sup>55</sup> cheap plaster-block. The glue, dextrine and silicate of soda may all be used in conjunction or separately or any combination of them may be added to the saw-dust, plaster-of-Paris and water according to the desired <sup>60</sup> effect to be produced.

While the above description has been restricted to using the composition for blocks obviously the composition may be applied directly to a wall, ceiling or partition in <sup>65</sup> the same manner as plaster is applied.

If desired I may incorporate in my composition cork in a finely divided condition. When using cork a less quantity of saw-dust is used and the proportions would then be <sup>70</sup> about one-half part of saw-dust, about one-half part cork to about one part of plaster-of-Paris. The glue, dextrine and silicate of soda may be added, if desired, in the proportions herein before mentioned.

What I claim is:—

A plaster block composition comprising approximately from a half to one part of saw dust mixed with about one part of plaster-of-Paris, there being added about one <sup>80</sup> part of water to wet the mixture, said water containing about 5% of liquid glue, about 5% of dextrine, and about 10% of silicate of soda.

In testimony whereof I have hereunto <sup>85</sup> signed my name.

FREDERICK M. VENZIE.